

1

Patent Drawing or Right-Handed Drawing  
3,661,823

## POLYFLUOROHYDROCARBON RESIN COMPOSITIONS AS CUSHION AND COVER COMPOSITIONS FOR V-BELTS

Sidney R. Fix, Stanley W. Olson, and John C. Wolfe, Lincoln, Nebr., assignors to The Goodyear Tire & Rubber Company, Akron, Ohio  
No Drawing. Original application Feb. 6, 1968, Ser. No. 703,248, now Patent No. 3,541,872, dated Nov. 24, 1970. Divided and this application Apr. 22, 1970, Ser. No. 38,643

Int. Cl. C08d 13/00

U.S. Cl. 260—17.4 BB

5 Claims

### ABSTRACT OF THE DISCLOSURE

V-belts containing the cushion compositions and/or elastomeric impregnated fabric envelopes which contain polyfluorohydrocarbon resins which increase the resistance to failure due to flexing of said V-belts.

This application is a division of application S.N. 703,248, filed Feb. 6, 1968, and now U.S. Pat. 3,541,872.

This invention relates to cushion stocks for V-belts, elastomeric impregnated fabric envelopes for V-belts, V-belts containing said cushion stocks and fabric envelopes, and a process for improving the resistance to failure due to flexing of said V-belts.

In the art of power transmission V-belts characterized by a cross section in the form of a trapezoid or truncated V which wedgingly engages the similarly shaped peripheral groove of a V pulley are employed in an ever increasing number of applications. A primary reason for this popularity is the improved load carrying and power transmitting capability afforded by the forced contact between the sides of the belt and the sides of the pulley groove which resist slippage of the belt in the pulley. These well known belts are normally characterized by such basic elements as a tension member composed of a rubber insulated cord layer, and a compression (cushion) section. An example of a belt of this type is described and illustrated (FIG. 3) in U.S. Pat. 3,051,212. Often the belt is covered by a rubberized fabric envelope which covers the entire surface of the belt. An example of such an envelope is discussed and shown in U.S. Pat. 3,260,126. In other instances no envelope is used, resulting in what is commonly known as a molded or raw edge belt. As a result of the severe operating conditions to which V-belts are often subjected, the resistance of the belts to failure due to flexing has become increasingly important. In addition, where the cushion section of the belt is not covered by a rubberized fabric the surface of the cushion after vulcanization can possess imperfections which not only detract from the appearance of the cushion section, but in addition, provide sites for flex cracking and other forms of deterioration to occur. It is therefore desirable to improve the performance and appearance of V-belts. It is desirable that the resistance to failure due to flexing be improved. Such failure can take the form of delamination of the elements of the belt and cord separation. Increased abrasion resistance is also desirable. It is also desirable to provide cushion sections with less surface imperfections in order to improve the appearance of the surface of the cushion stock and also to aid in preventing flex cracking and other forms of deterioration.

It is an object of the present invention to provide V-belts with improved resistance to failure due to flexing and improved abrasion resistance, cushion stocks and elastomeric impregnated fabric envelopes (fabric covers) which will aid in providing said V-belts with improved

2

resistance to failure due to flexing and aid in providing improved abrasion resistance, and a process for improving the resistance to failure due to flexing and to improve the abrasion resistance of V-belts.

Some of the objects of the present invention are accomplished by blending a carbon black loaded composition comprising (A) 100 parts by weight of at least one elastomeric compound comprising (1) from about 50 to 100 parts by weight per 100 parts by weight of the elastomeric compound of polychloroprene and (2) from 0 to about 50 parts by weight per 100 parts by weight of the elastomeric compound of at least one rubbery diene polymer, (B) from about 0 to about 75 parts by weight per 100 parts by weight of the elastomeric compound of at least one flexible filamentary material and (C) from about 0.5 to about 20.0 parts by weight per 100 parts by weight of the elastomeric compound of at least one polyfluorohydrocarbon resin and then building a V-belt using the above composition to form the cushion portion of the belt and vulcanizing said V-belt. Some objects are accomplished by impregnating fabric with the above composition to form fabric envelopes for V-belts. Other objects will appear subsequently herein.

Preferably the elastomeric compound consists essentially of polychloroprene, i.e., the rubbery polymer of 2-chlorobutadiene-1,3. This material is designated as ASTM D 1418-56T at (C).

Rubber diene polymers which may be used in combination with the polychloroprene include natural rubber, such as crepe rubber, and synthetic rubbers such as homopolymers of a conjugated 1,3-diene such as isoprene and butadiene, and in particular, polyisoprenes and polybutadienes having essentially all of their repeating units combined in a vis-1,4 structure; copolymers of a conjugated 1,3-diene such as isoprene and butadiene with up to 50 percent by weight of at least one copolymerizable monomer such as styrene and acrylonitrile; and polymers of monoolefins containing unsaturation, i.e., carbon to carbon double bonds, such as terpolymers of ethylene, propylene and a nonconjugated diene.

The flexible filamentary material to be used in the practice of the present invention may be any flexible fiber of a shortened length which is generally used to increase the stiffness and hardness of cushion stocks. Such usage of fibers is noted in U.S. Pat. 3,051,212, column 4, lines 67 and 68. Well known fibers such as cotton linters and chopped or ground polyamides, such as nylon, regenerated cellulose such as rayon; and polyester fibers are exemplary of the types of the materials that may be used as flexible filamentary materials. The materials should be of such size that they can be dispersed uniformly throughout the cushion stock, and of such size to provide an increase in stiffness and hardness of the cushion stocks. Preferably from about 5 to about 30 parts by weight of the flexible filamentary material are used.

Polyfluorohydrocarbon resins, which have polymer lubricating properties, which may be used in the practice of the present invention are essentially completely fluorinated polymers such as polytetrafluoroethylene and essentially completely fluorinated ethylene propylene copolymers such as those made by copolymerizing hexafluoropropylene and tetrafluoroethylene. Preferably from about 1.0 part to about 5.0 parts of the polyfluorohydrocarbon resin are used per 100 parts by weight of the elastomeric compound. It is preferred that the polymers be in powdered form to facilitate ease of incorporation into the elastomers with conventional mixing equipment.

The method of combining the components of the cushion stock is not normally critical. The elastomeric compound, flexible filamentary material and polyfluorohydrocarbon resin may be mixed by such methods as Banbury

mixing and open mill mixing. The components may be mixed in any order, in increments, and in any combination.

Any conventional vulcanization system may be used to vulcanize the cushion stock. When the elastomeric compound of the cushion stock consists essentially of poly-chloroprene, materials such as zinc oxide may be used to vulcanize the cushion stock. Where diene polymers are used as a portion of the elastomeric compound it is preferred that some sulfur vulcanization system be used.

Any conventional carbon black may be used to load the cushion stock. The level of black should normally be from about 10 to about 90 parts by weight per 100 parts by weight of the elastomeric compound. A range of from about 20 to about 40 parts by weight is preferred.

The cushion stock composition may also be used to impregnate fabric to form fabric envelopes for V-belts, with the qualification that it preferably contains essentially no fiber loading. An example of a fabric envelope for a V-belt is shown in FIG. 6 and discussed at column 5, lines 26 to 28 of U.S. 3,260,126. The fabric may be any conventional V-belt fabric, e.g., cotton, rayon, nylon and polyesters. The fabric may be impregnated in any conventional manner, for example by swelling the elastomer in an organic solvent to form a dough-like composition, spreading the dough-like composition on the fabric and driving off the organic solvent. Said envelopes improve the resistance to failure due to flexing of V-belts.

The following examples contain illustrations of the practice of the present invention and are not intended to limit the present invention.

#### EXAMPLE 1

Eight V-belts, A through H, having tensile and cushion elements were fabricated using identical trapezoid type construction and vulcanized. The cushion portions of the belts were devoid of any fabric envelopes. The compounds and cords used in constructing the V-belts were the same with the exception of the cushion portion of the belts. The cushion portion of belts A through D was prepared by milling together the following formulation.

| Components:                            | Parts by weight |
|----------------------------------------|-----------------|
| Nonproductive polychloroprene stock    | 64.50           |
| Scrap                                  | 25.00           |
| Zinc oxide                             | 3.50            |
| Chopped cotton, rayon and nylon fibers | 7.00            |

The cushion portion of belts E through H was prepared by milling together the following formulation.

| Components:                          | Parts by weight |
|--------------------------------------|-----------------|
| Nonproductive polychloroprene stock  | 45.80           |
| Scrap                                | 50.00           |
| Zinc oxide                           | 3.53            |
| Polytetrafluoroethylene <sup>1</sup> | 0.67            |

<sup>1</sup> Teflon, TL=115.

The nonproductive polychloroprene stock contained 100 parts by weight of polychloroprene as its sole elastomeric component, 20.0 parts of FEF carbon black, magnesium dioxide, processing oil, stearic acid, phenylbetanaphthylamine and phenylalphanaphthylamine.

The scrap was unvulcanized productive V-belt scrap which had been ground into fine particles. The scrap V-belts were similar to belts A through H regarding both construction and composition. However, the cushion portion did not contain polytetrafluoroethylene. The insulation portion of the V-belt scrap comprised approximately 20 percent by weight of the V-belt scrap. The polyester cord comprised about 5 percent by weight. The cushion portion comprised about 75 percent by weight. The insulation portion contained 100 parts by weight of polychloroprene as its sole elastomeric component, 20.0 parts of FEF black, 10.0 parts of cotton linters, reinforcing silica,

magnesium oxide, processing oil, stearic acid, zinc oxide, a polyethylene-wax-releasing-agent-and-phenylalphanaphthylamine.

As mentioned above, the cushion portion of the V-belt scrap had approximately the same composition as the cushion stocks of belts A to H. The cushion stocks in belts A to H were essentially the same, containing approximately 15 percent by weight of chopped fiber, with the exception that the cushion portion of belts E to H contained polytetrafluoroethylene and the cushion portions of belts A to D contained no polytetrafluoroethylene. Both sets of belts contained a tensile portion comprised of polyester cords insulated by an elastomeric formulation similar to the insulation composition described earlier herein.

#### EXAMPLE 2

Cushion stocks for V-belts within the scope of the present invention are also prepared by mixing the following compounds on an open mill.

| Components:             | Parts by weight |
|-------------------------|-----------------|
| Polychloroprene         | 100.0           |
| Carbon black (FEF)      | 30.0            |
| Magnesium oxide         | 2.0             |
| Processing oil          | 7.5             |
| Amine antioxidant       | 0.50            |
| Stearic acid            | 1.0             |
| Wax                     | 2.0             |
| Cotton linters          | 15.00           |
| Polytetrafluoroethylene | 2.00            |
| Zinc oxide              | 4.00            |

Chopped or ground rayon, nylon and polyester fibers are interchangeable with cotton linters. Other essentially completely fluorinated polyfluorohydrocarbon resins such as essentially completely fluorinated ethylene propylene copolymer are also interchangeable with polytetrafluoroethylene.

#### EXAMPLE 3

The belts of Example 1 were dynamically tested on a pulley arrangement according to SAE procedure J 637 (SAE Handbook, 1967 edition), at 13 horsepower with the exception that the small pulley was 2.5 inches in diameter. The time to first failure as indicated by the first parting of any of the elements of the belt from the rest of the belt was recorded.

| Belt: | Condition of belt at failure | Time to failure (hours)                                    | Time to failure |     |     |     |
|-------|------------------------------|------------------------------------------------------------|-----------------|-----|-----|-----|
|       |                              |                                                            | 1               | 2   | 3   | 4   |
| 50    | A                            | Components separated at cordline, top fabric came off.     | 159             |     |     |     |
|       | B                            | Top fabric came off, edge cord came out side of belt.      |                 | 166 |     |     |
|       | C                            | Top fabric came off, edge cord came out side of belt.      |                 |     | 238 |     |
| 55    | D                            | Cushion section delaminated from rest of belt.             |                 |     |     | 246 |
|       | Average                      |                                                            |                 |     |     | 302 |
| 60    | Belt:                        |                                                            |                 |     |     |     |
|       | E                            | Delamination of insulation to cordline.                    |                 |     |     | 369 |
|       | F                            | Severe delamination at cordline.                           |                 |     |     | 336 |
|       | G                            | Delamination at cordline.                                  |                 |     |     | 366 |
|       | H                            | Edge cord broke outside of belt; delamination at cordline. |                 |     |     | 256 |
|       | Average                      |                                                            |                 |     |     | 282 |

As shown by the above data the belts possessing a cushion within the scope of the present invention (belts E to H) possessed a resistance to failure due to flexing which was superior to the resistance of belts outside the scope of the present invention (belts A to D).

The surfaces of the cushion portions of belts A to D also contained some surface imperfections, whereas the surface of the cushion portions of belts E to H contained no appreciable surface imperfections.

The belts tested in Example 3 did not possess a fabric envelope surrounding the cushion element. Tests, however, have been run with belts containing a cushion ele-

ment surrounded by a fabric envelope. The cushion element contained polytetrafluoroethylene. These belts also showed improved resistance to failure due to flexing. The use of polyfluorohydrocarbon resins also enhances the abrasion resistance of the cushion stocks.

#### EXAMPLE 4

Eight V-belts (I through P) were constructed in essentially the same fashion as the belts A to D described in Example 1 and vulcanized. The composition of the elements was similar to the composition of the elements of belts A to D. The construction of the belts differed in that each belt contained a fabric envelope (cotton/nylon blend) impregnated with a black loaded (50 parts by weight of black) productive polychloroprene stock. The fabric was impregnated by swelling the polychloroprene composition with an organic solvent to form a dough-like composition, spreading the dough-like composition on the fabric and driving off the solvent. The cushion stock of these eight belts did not contain fiber loading. Four belts (M to P) contained polytetrafluoroethylene in the polychloroprene portion of the fabric envelope, also known as a fabric cover. The other four belts (I through L) contained no polytetrafluoroethylene in the fabric envelope. The belts were tested in a manner similar to that described in Example 3 using a 2.5 idler pulley, a tension of 140 pounds and 14 horsepower.

| Belt:   | Time to failure<br>(hours) |
|---------|----------------------------|
| I       | 44                         |
| J       | 69                         |
| K       | 96                         |
| L       | 76                         |
| Average | 71                         |
| M       | 112                        |
| N       | 94                         |
| O       | 76                         |
| P       | 131                        |
| Average | 103                        |

As shown by the above data, belts M through P of the present invention were superior in performance.

The use of polyfluorohydrocarbon resins also enhances the abrasion resistance of the fabric envelopes.

While certain representative embodiments and details have been shown for the purpose of illustrating the invention it will be apparent to those skilled in this art that various changes and modifications may be made therein without departing from the spirit or scope of the invention.

What we claim is:

1. An elastomeric composition comprising (A) 100 parts of at least one elastomeric compound having (1) from about 50 to 100 parts of polychloroprene and (2) from about 0 to about 50 parts of a different rubbery diene polymer; (B) from about 5 to about 30 parts of at least one flexible filamentary material; (C) from about 0.5 to about 20.0 parts of at least one polyfluorohydrocarbon resin selected from the group consisting of polytetrafluoroethylene and essentially completely fluorinated ethylene propylene copolymer resins; and (D) from about 10 to about 90 parts of carbon black, said parts being by weight per 100 parts of elastomeric compound.
- 10 2. A composition according to claim 1 wherein the elastomeric compound consists essentially of polychloroprene.
- 15 3. A composition according to claim 1 wherein the flexible filamentary material is selected from the group consisting of a polyamide, regenerated cellulose, polyester and cotton.
- 20 4. A composition according to claim 1 wherein the polyfluorohydrocarbon resin is polytetrafluoroethylene.
- 25 5. A composition according to claim 3 wherein the amount of polyfluorohydrocarbon resin is from about 1.0 to about 5.0 parts.

#### References Cited

##### UNITED STATES PATENTS

- |           |         |        |           |
|-----------|---------|--------|-----------|
| 3,002,938 | 10/1961 | Gagne  | 260—890 X |
| 3,011,221 | 12/1961 | Howell | 260—890 X |
| 3,223,676 | 12/1965 | Rucker | 260—890 X |

WILLIAM H. SHORT, Primary Examiner

40 L. L. LEE, Assistant Examiner

U.S. Cl. X.R.

74—233; 260—57 R, 873, 890